

July 2, 1946.

H. B. LAW

2,403,225

METHOD OF MANUFACTURING ELECTRODE FOUNDATION STRUCTURES

Filed April 29, 1943

Fig. 1.



Fig. 3.



Fig. 2.



Fig. 4.



Fig. 5.



INVENTOR

BY HAROLD B. LAW  
*Charles McClain*  
ATTORNEY

Patented July 2, 1946

2,403,225

# UNITED STATES PATENT OFFICE

2,403,225

## METHOD OF MANUFACTURING ELECTRODE FOUNDATION STRUCTURES

Harold B. Law, Princeton, N. J., assignor to Radio Corporation of America, a corporation of Delaware

Application April 29, 1943, Serial No. 485,048

7 Claims. (Cl. 49—79)

1

My invention relates to television transmitting tubes and electrode structures and more particularly to improved methods of manufacturing target structures suitable for use in tubes of the low velocity electron beam scanning and electron image types.

In my prior application Serial No. 463,065, filed October 23, 1942, of which this application is a continuation-in-part, I described a target electrode wherein an imperforate sheet of vitreous material was provided with a great number of recesses, the sheet being etched to provide a corresponding number of apertures which might be used as image grid apertures or filled with conductive material to form a mosaic electrode. In my prior structure the recesses or apertures as formed were nonuniformly distributed over the surface of the foundation sheet. This offered a disadvantage in that without a symmetrical array of recesses or apertures the degree of resolution obtainable when such a target is used in a television tube is not as high as desired and cannot be maintained uniform from tube to tube.

It is an object of my invention to provide target structures for electron beam tubes such as of the television transmitting type whereby higher sensitivity and lower distortion than those obtainable with prior structures may be obtained. It is a further object to provide a method whereby such structures may be manufactured with ease and at low cost. It is a further object of my invention to provide methods of manufacturing electron beam targets having a uniform array of discrete mosaic areas, and it is a still further object to provide a target electrode and method of manufacture which may be duplicated with a high degree of accuracy so that uniform characteristics from tube to tube may be obtained. In accordance with my invention I provide a thin sheet of imperforate vitreous insulating material and provide on said sheet by photographic processes a tacky discontinuous surface to which very fine particles of silicon carbide are made adherent, followed by firing the sheet and particles at an elevated temperature to provide recesses or bubbles distributed as a uniform array over the surface of the sheet. As disclosed in my original application, I may form apertures over the recessed or bubble area of the vitreous sheet by acid etching whereupon, for specific uses and in accordance with my invention, I fill the apertures with metal without coating adjoining surfaces of the sheet with conductive matter remaining after the sheet is ready for use. Alternatively, the apertures may be coated with

2

mosaic particles only over the internal surfaces or over the boundary areas thereof, thereby forming an image grid type electrode.

These and other objects, features and advantages of my invention will be apparent from the following description and with reference to the accompanying drawing wherein:

Figure 1 shows a portion of a vitreous foundation sheet partially prepared for use in practicing my invention, and

Figures 2-7 show various stages of the manufacturing process in accordance with my invention.

It will be appreciated that the target structure made in accordance with my invention is useful in many types of electron discharge tubes, particularly of the television transmitting and image recreation types, and consequently, I have not shown in the drawing any particular type of tube to which it is applicable. For example, the target structure may be utilized in image tubes scanned by a low velocity electron beam such as described in U. S. Patent 2,213,179, although one modification thereof may be used as a double-sided mosaic electrode as shown in U. S. Patent 2,213,178. In addition, an electrode made in accordance with my invention may be used as an electron emission image control electrode such as described in my copending application Serial No. 463,066, filed October 23, 1942. While the final target electrodes as used in these various tubes are somewhat different by reason of additional processing, my method of manufacture provides an electrode or electrode foundation suitable for such use with or without additional processing steps as disclosed more particularly hereinafter.

Referring to Figure 1, the target foundation comprises a very thin initially imperforate foundation sheet 1 of electrically insulating or semi-insulating material such as glass having a resistance, for the particular applications referred to below, greater than  $10^{11}$  ohm-centimeters. Preferably, an exceptionally thin homogeneous sheet of glass having the desired specific resistance dependent upon its specific use and being smooth and of uniform thickness may be used. I have used glass known in the art as Corning 705 glass with satisfactory results. Preferably, the target foundation sheet 1 has an initial thickness of from 0.001 to 0.005 inch and may be provided by blowing a bubble of the desired glass composition, the wall of the bubble then being sealed and flattened on an annular flanged support 2, as described by Albert Rose in his co-

pending application Serial No. 407,131, filed August 16, 1941.

I will describe two alternate steps for preparing the foundation sheet 1, the results of which I have shown in Figures 2 and 3 respectively. Referring to Figure 2 and following one of these alternate steps, I coat the upper surface of the thin foundation sheet 1 shown in Figure 1 with a thin coating of a tacky substance, such as a very thin coating of rubber cement 3. The prerequisites of this coating are that it should be tacky, adhesive and preferably of volatile material so that upon a subsequent operation it may be removed such as by baking at an elevated temperature. The thin coating 3 of rubber cement 15 may be formed of latex dissolved in a latex solvent, and I have found the commercial rubber cement known as "Best-Test" as supplied by the Union Rubber and Asbestos Company, of Trenton, New Jersey, most suitable for the purpose. The rubber cement is applied in fairly liquid form so that it may spread over the entire upper surface of the foundation sheet 1 and then allowed to dry for a few minutes. Following the application of the tacky coating 3 and as shown in Figure 2, I then provide on the coating 3 a photographic emulsion 4 which may be a layer of gelatin containing potassium dichromate. I have obtained excellent results using a proportion of 3.3 grams of photographic quality gelatin with 12 cubic centimeters (cc.) of 4% potassium dichromate solution and sufficient water to provide 100 cc. of solution. Preferably, I add a few drops of a commercial wetting agent such as Aerosol to the solution so that upon flowing the solution over the exposed surface of the coating 3 the gelatin solution adheres thereto and forms the layer of photographic emulsion 4 shown in Figure 2. Obviously, the preparation of the photographic emulsion is preferably performed in subdued light so as to prevent undue exposure of the potassium dichromate in the solution and in the resultant emulsion 4. I then expose the photographic emulsion 4 through a negative of an electrolytic screen that is, through the negative of a series of crossed parallel closely spaced opaque lines thereby shielding from exposure uniformly separated point-like areas over the surface of the emulsion. As shown in Figure 2, I provide a light transparent negative foundation 5 having uniformly separated point-like opaque areas 6 so that the emulsion 4 may be exposed from a light source X through the areas 7 forming in effect a uniform exposure of crossed parallel closely spaced lines over the surface of the emulsion. I then develop the exposed emulsion 4 in water at about 50° C. which removes the gelatin of the emulsion not exposed over the point-like opaque areas and hardens the remaining gelatin so that it loses its tackiness. As a result of this step, the tacky coating 3 is physically exposed to the atmosphere by the removal of the gelatin over the areas previously photographically unexposed and removed by washing, whereas surrounding areas of the emulsion 4 are retained on the tacky coating 3.

Following the preparation of the foundation, I dust very fine silicon carbide into the apertures formed in the emulsion coating and into contact with the tacky coating 3, the excess being blown off with a blast of air leaving isolated piles of silicon carbide in the apertures formed in the emulsion 4. Referring to Figure 4, I have shown small piles 8 of silicon carbide separated by the hardened emulsion lines 9.

Another alternative method of preparing the foundation sheet 1 is shown in Figure 3 wherein the sheet 1 is coated directly with the photographic emulsion 4', this emulsion being rendered tacky for the purpose of attaching silicon carbide particles, thereby serving a dual purpose, namely, as a photographic emulsion and as the tacky coating 3. In this modified step of my process, however, I use a photographic emulsion solution which when dry is inherently tacky so that the silicon carbide may be distributed uniformly and become uniformly adherent to the emulsion layer as shown in Figure 3 at 10; for example, the silicon carbide particles may be applied by depositing a quantity thereof on the emulsion 4', the excess particles being blown off with a blast of air. Following the application of the silicon carbide particles, the emulsion layer 4' is exposed to light, such as from the light source X shown in Figure 3, through a positive 6a of an electrolytic screen and through the foundation sheet 1 inasmuch as the silicon carbide particles are relatively opaque rendering projection through the sheet 1 necessary. It will be noted that this exposure exposes minute half-tone dot-like areas of the emulsion which is then developed in water to remove the unexposed emulsion. This development is preferably in hot water, approximately 50° C., the temperature being proportional to the time of exposure. Following this washing process, the foundation sheet 1 will have small discrete separated areas of the emulsion supporting the silicon carbide particles, these areas being separated by clear areas of the foundation sheet from which the emulsion and the silicon carbide particles have been removed.

It will be noted that in using either of the steps which I have described above the foundation sheet 1 is provided with mutually separated piles of silicon carbide particles, separated from the foundation in the first instance by the tacky rubber film 3, and in the second instance by individual areas of the photographic emulsion. The prepared foundation is then fired or baked at a temperature slightly exceeding the softening point of the vitreous foundation. During the initial stages of this baking the rubber coating 3 or the remaining areas of the emulsion 4, as the case may be, vaporize and small bubbles 11 are formed in the vitreous foundation sheet 1 as shown in Figure 5. Preferably, this firing or baking step is performed by placing the prepared foundation sheet in a furnace or oven at room temperature and heating the oven and sheet to a final temperature at which the foundation slightly softens. This temperature will depend upon the particular composition of the foundation sheet, although when using the 705 glass referred to above the bubbles 11 begin to form at a temperature around 775° C. Alternatively, using this same glass the prepared foundation may be inserted in an oven which has been heated previously to approximately 800° C., allowing the foundation to remain in the oven for 5 minutes following which it is removed from the oven and cooled. If glass other than Corning 705 is used, the required baking temperature may vary slightly from the above temperature and I have found that a temperature at which the glass sticks and seals to the iron-nickel-cobalt alloy described by Scott in his U. S. Patent 1,942,260 is a satisfactory temperature for forming the bubbles 11. I have been unable to discern any difference in the bubbles whether or not use is made of the rubber film intermediate the emul-

sion and the glass, or whether the photographic emulsion alone is used, the bubbles appearing to be substantially the same size and configuration notwithstanding which alternative step is used.

Following the firing operation I immerse the sheet in a hydrofluoric acid solution which loosens and dissolves the silicon carbide particles as well as a portion of the glass foundation. Consequently, the thickness of the original glass foundation sheet is chosen to allow for this step and 10 consequent reduction in sheet thickness. For this step I prefer to use an aqueous solution of ten parts of water to one part of concentrated hydrofluoric acid. The foundation may be immersed in this solution for a time sufficient to 15 remove the silicon carbide particles but insufficient to open the bubbles to the lower side of the foundation sheet leaving the sheet in its imperforate form as shown in Figure 5. Such a foundation is of particular advantage in my second-mentioned copending application wherein the lower surfaces of the bubbles 11 are provided with a red sensitive photo-electric coating, the upper surface of the sheet, that is around the recesses or bubbles, being coated with a blue sensitive photo-electric coating. Alternatively, the foundation shown in Figure 5 may be allowed to remain in the acid solution for a time sufficient to 20 open the bubbles on the lower side to provide the structure shown in Figure 6 wherein the bubbles have formed apertures 12 extending completely through the foundation sheet 1. Such a structure is useful when coated on one side with a mosaic of photosensitive elements for use in a tube such as shown by U. S. Patent 2,213,179. Further in accordance with my invention, the apertures 12 shown in Figure 6 may be filled with 25 metal plugs 13 to provide a target of the double-sided type such as shown in Figure 7. To provide this type of target I lay a thin lacquer film over one surface of the foundation following the acid treatment and following the opening of the apertures 12 through the foundation. Such a thin lacquer film may be produced by allowing a drop 30 of lacquer to spread over the surface of an immiscible liquid such as water. The lacquer, following spreading, dries very rapidly and the thin film may be placed on the foundation 1 by immersing the foundation in the water prior to 35 formation of the film and withdrawing the foundation thereby lifting the lacquer film upon the apertured foundation and from the surface of the water. The apertures are then filled with a 1% gelatin solution from the opposite side of the foundation from the lacquer film. This filling of 40 the apertures may be performed by first pouring the gelatin solution upon the foundation and then draining and drying, these alternate steps being repeated several times. I then dissolve the lacquer film by immersing the foundation in acetone or other solvent for the lacquer and replace the film with a conducting layer such as a film of graphite or aluminum. If graphite is used, it may be spread on the surface following removal of the lacquer. Or if a metal such as aluminum is used, it may be vaporized and condensed on this surface. Following the application of the conductive film, the gelatin filling the apertures is removed by immersing the treated foundation in hot water. The graphite or metal coating is then used as a cathode for silver plating to fill the apertures with silver to form the silver plugs 13 as shown in Figure 7. To provide these silver plugs a conventional silver plating solution may be poured into the apertures, that is, from the 45

side from which the gelatin was removed, whereupon the silver is electrolytically plated on the graphite or aluminum film portions exposed through the apertures 12, using the conducting layer of graphite or aluminum as a cathode. Following the formation of the silver plugs, the conducting film, if of graphite, is removed by use of a solvent for the graphite binder, or by dissolving in sodium hydroxide if the film is made of aluminum.

Alternatively, the metal plugs 13 may be formed in the apertures of the foundation by a somewhat modified process wherein the thin lacquer film, as previously described, is laid upon the apertured foundation followed by the application of graphite directly thereto for the formation of a conductive film. I prefer to mix graphite with wood alcohol to a relatively thin consistency and brush this mixture on the lacquer film. The wood alcohol serves as a partial solvent to wet the lacquer, forming electrically conductive paths through the lacquer film to the graphite coating. After this coating is dry I place the graphite in contact with a mercury bath and pour the plating solution over the bath to fill the apertures with the plating solution. The mercury bath and graphite coating then serve as a cathode in the plating operation, forming the mutually separated metal plugs in the foundation 1.

From the above, it will be appreciated that I have provided accurate means for distributing minute piles of silicon carbide over the surface of a thin glass foundation and using these piles to provide under the influence of heating a corresponding number of bubbles or apertures distributed in the same order over the foundation sheet and likewise a new method of developing metal plugs within the apertures thus formed. Furthermore, while I have disclosed only three specific types of electron discharge tubes in which my electrode structure is applicable, it will be appreciated that the structure may be used in other tube types and for other applications than the specified television transmitting and image tube use without departing from the scope of the appended claims.

I claim:

1. The method of manufacturing a foundation for an electrode structure comprising forming discrete separated adhesive areas on a glass foundation, distributing fine particles of silicon carbide over said adhesive areas and heating said foundation to a temperature sufficient to soften said glass and form bubbles in said foundation underlying said adhesive areas by said gas.

2. The method of manufacturing a foundation for an electrode structure comprising distributing fine particles of silicon carbide over separated adhesive areas on a glass foundation, and heating said foundation and said particles to a temperature approximating the softening temperature of said glass to form bubbles underlying said fine particles of refractory material by said gas and removing said particles to expose said bubbles.

3. The method of manufacturing an electrode foundation structure comprising forming discrete uniformly separated adhesive areas on a glass foundation, covering each of said areas with a quantity of fine particles of silicon carbide, heating said glass foundation bearing said particles to a temperature approximating the softening point of said glass to form bubbles in said glass underlying said particles and removing said particles to expose a regular array of bubbles posi-

tioned in accordance with the uniform separation of said areas.

4. The method of manufacturing an electrode foundation structure comprising the steps of coating a thin glass sheet with an adhesive layer, coating said layer with a photographic emulsion, exposing portions of said emulsion to light through a photographic negative thereby shielding uniformly separated point-like areas of said emulsion from light, developing and washing said emulsion to expose to view uniformly separated point-like areas of said adhesive, coating said point-like adhesive areas with particles of silicon carbide and baking said foundation to develop bubbles therein over said point-like areas.

5. The method of manufacturing an electrode foundation structure comprising the steps of forming an adhesive coating on a thin glass foundation, covering said coating with a mask of photographic emulsion, exposing and developing predetermined portions of said emulsion to unmask portions of said coating, covering said portions of said coating with fine particles of silicon carbide, heating the prepared foundation to a temperature at which the glass softens and at which bubbles are formed therein, and immersing said foundation in an acid to remove said particles of silicon carbide.

6. The method of manufacturing a target elec-

trode member comprising a thin sheet of glass comprising coating said sheet of glass with an adhesive film of photographic emulsion of the potassium dichromate type, covering said film with fine particles of silicon carbide, exposing portions of said film to light, removing the portions thereof not exposed together with the overlying silicon carbide particles, heating the prepared sheet of glass to develop bubbles in said glass sheet underlying the remaining particles of silicon carbide and removing the remaining particles of silicon carbide to expose said bubbles at the surface of said sheet of glass.

7. The method of manufacturing an electrode foundation structure comprising coating a thin sheet of glass having a softening point below 800° C. with a photographic emulsion film containing an adhesive substance, coating said film with fine particles of silicon carbide, photographically exposing said emulsion through said sheet of glass over separated point-like areas, removing the unexposed portions of said emulsion while retaining said particles on the exposed portions thereof and heating the prepared sheet of glass to a softening temperature to develop bubbles underlying the particles of silicon carbide retained on the exposed portions of said emulsion film.

HAROLD B. LAW.